

Sept. 20, 1938.

R. FORSYTH

2,130,681

PROCESS AND APPARATUS FOR DERIVING FIBER FROM FLAX STRAW OR THE LIKE

Original Filed July 23, 1931 2 Sheets-Sheet 1



Sept. 20, 1938.

R. FORSYTH

2,130,681

PROCESS AND APPARATUS FOR DERIVING FIBER FROM FLAX STRAW OR THE LIKE

Original Filed July 23, 1931 2 Sheets-Sheet 2



Inventor:  
Robert Forsyth.  
by ~~Robert~~ ~~Robert~~  
his Attorneys.

## UNITED STATES PATENT OFFICE

2,130,681

PROCESS AND APPARATUS FOR DERIVING  
FIBER FROM FLAX STRAW OR THE LIKERobert Forsyth, Chicago, Ill., assignor to Robert  
N. Burton, Chicago, Ill.Application July 23, 1931, Serial No. 552,618  
Renewed November 7, 1936

7 Claims. (Cl. 19—7)

This invention relates to a process and to apparatus for performing the process of separating or deriving from certain vegetable stalks or stems the fibrous structure thereof in the form of individual fibers. Such fibrous material is adapted for use in the textile art for spinning and weaving thread and cloth in the nature of linen; it is also valuable for the manufacture of certain grades of paper commonly known as 10 "bond" paper and for the paper stock employed for currency; another and quite different use for such fiber is for packing or wicking for which it is suitable by reason of its capillary structure and in which capacity it may replace the cotton 15 waste commonly employed for packing journal bearings like those of railway car axles. These are only a few examples of the range of uses of such fiber. The process is designed and illustrated with respect to the treatment of threshed 20 flax straw, or like material, in such manner that the entire straw can be made available for use by separation into its component parts including the woody portion or shive, the gum and resin, the tannin and chlorofyl and the fiber itself.

25 An object of the invention is to provide a process and apparatus for mechanically accomplishing this purpose; another object is to insure a relatively gentle treatment of the fiber throughout the process so that it shall retain all of its original tensile strength and other desirable qualities without the impairment which might result from excessive chemical treatment or rough mechanical handling; another object is to maintain the fibers as far as possible in their original unbroken length and in substantial alignment through 30 the process to avoid tangling and breakage; and it is also an object of the invention to provide a substantially continuous process adapted to operate on a definite time schedule whereby a given 35 plant may be depended upon to turn out a known quantity of finished fiber in a given time with the various steps of the process under definite control at all times. Other objects will appear 40 as the description proceeds. The invention 45 therefore consists in the various steps of the process in combination and in certain features and elements of the apparatus and the relative arrangement of the parts thereof, all as hereinafter 50 described and shown in the drawings and as indicated by the claims.

Figure 1 is a diagrammatic side elevation of the apparatus for the initial steps of the process including a feeding belt, flattening rolls and additional rolls for flexing the straw and a picker

of typical construction, all for treating the straw in the dry state.

Figure 2 illustrates diagrammatically in vertical section the first series of troughs in which the fiber is treated for softening the gums and 5 resins and also squeezing rolls associated with said troughs, together with a portion of the second series of troughs from which the material is fed from the rolls.

Figure 3 is in effect a continuation of Figure 2 10 showing the terminal portion of the second set of troughs with additional squeezing rolls and also a neutralizing acid bath, a rinsing water bath, the final squeezing rolls, a traveling dryer belt and a set of rolls for mechanical softening 15 of the dry fiber.

Figure 4 is a diagrammatic detail mainly in section, showing the corrugations of the flexing rolls illustrated in Figure 1, and including 20 one of the hook shaped picker teeth to which said rolls feed the straw.

Figure 5 is a transverse section of one of the tanks or trough assemblies, being taken substantially as indicated at line, 5—5, on Figure 2.

Figure 6 is a detail elevation of the squeezing 25 rolls shown in Figure 2.

Figure 7 is a detail section on a larger scale showing the construction of the troughs of Figure 5.

Figure 8 is a partial plan view of said troughs. 30

This process having been designed primarily for the treatment of flax stalks or straw and particularly for handling threshed flax straw, will be described with reference to that material although it may be understood that the process 35 may be suitable wholly or in part for deriving the fibrous content of other similar plant growths. It may be understood that the process is designed primarily to employ the straw shortly after the threshing process has been completed, 40 but preferably with the straw thoroughly dried. That is, it is not intended or contemplated that the straw shall be retted as was once the practice, by permitting it to partially rot on the ground or under water to allow deterioration of 45 the wood portion, since such treatment has a tendency to deteriorate and weaken the fiber itself as well as to waste the woody material or shive which itself has a definite value, as for use in various wood pulp products, including news 50 print.

Assuming then that the straw is supplied in a dry condition, it is fed by any convenient means such as by a conveyor belt, 1, for delivery between a pair of plain rolls, 2, 2, which serve to 55

flatten the straw and tend to split the fibers apart to some extent, and partially break up the woody material adhering to them. For further loosening this material, the straw passes directly between several pairs of fluted rolls whose grooves or corrugations are smoothly rounded and extend longitudinally, that is, parallel to the axes of the rolls and without any sharp edges. Four pairs of such rolls are shown at 3, 4, 5 and 6 in Figure 1, and from Figure 4 it may be noted that these rolls are designed to operate so that the flutings of each pair are intermeshed with each other but with clearance space between them, and it may be further observed that the rolls are disposed in a graduated arrangement such that the flutings of the rolls, 3, 3, are somewhat wider than the flutings of the rolls, 4, 4, and likewise the clearance space between the first pair of rolls is greater than that between the second pair, while the width of the flutings and the clearance space between the final pair of rolls, 6, 6, is the least in the series. The purpose of this arrangement is to cause the rolls to mildly flex the straw as it passes through them, tending to break the woody portions into short sections and to loosen them from the fibers themselves, this treatment being slightly more severe when the straw reaches the final set of rolls, 6, 6, than when it enters a set of rolls, 3, 3. As a result of this treatment the fibrous stalks shed a considerable portion of their woody content or "shive" before they reach the drum, 7, of the picker, 8, and are caught up by the hook-like teeth, 9, of said drum to be carried through the picker. This machine may be similar to those used for a like purpose and of generally standard construction, it being understood that its function is to comb the fibrous material by means of toothed rolls tending to split the fibers apart and straighten them out and at the same time serving to break off most of the remaining fragments and particles of the woody material or shive. Merely as a suggestion for the picker, 8, I have indicated in dotted outline two pairs of so-called "working" rolls at 18 and 19, and a final large delivery roll or drum, 11, by which it may be understood the fiber is discharged over a suitably inclined chute or table, 12, into a receiving basket or car, 13.

The dry fiber which is thus loosely piled or coiled in the receptacle, 13, may be accumulated as desired, as for example, until the receptacle is well filled, at which time the accumulated fiber will be definitely cut or broken off from that which continues to discharge from the picker, another receiving car or basket being placed in position and the first car being wheeled to the receiving end of the tank, 14, at A. The cut or broken ends of the fiber in the receptacle, 13, are bunched or assembled to form a "sliver" which may be started through the trough-like structure of the tank, 14, either by tying it with a string and leading the string through the feed rolls, 15, at the opposite end of the tank, 14, or by leading the "sliver" itself through the tank and starting its end portion through these rolls, 15. It is desirable, however, that the fiber shall experience a soaking treatment in the heated water bath of the tank, 14, for a period of at least thirty-five minutes; therefore, if the lead string is not employed, the sliver will be merely drawn through the length of the tank, 14, and allowed to lie there for this period before being started through the feed rolls, 15.

The tank, 14, as more clearly indicated in Figure 5 consists of outer side walls, 17, and a bottom wall, 18, within which are shown longitudinally

extending baffle walls, 19, spaced inwardly from the side walls, 17, with communication ports or openings, 20, in said baffle walls near the bottom. Near the top of the tank and below the upper edges of the side walls, 18, a series of longitudinally extending troughs, 21, are supported on any suitable framing, 22, and are provided with perforated bottoms, 23, as indicated in Figures 7 and 8. Steam pipes, 24, are shown supported adjacent the side walls, 17, and it may be understood that with the tank, 14, substantially filled with water the heating effect of the steam pipes will be to cause a circulation of the water upwardly between the side walls, 18, and their adjacent baffles, 19, and thence horizontally over the troughs, 21, and downwardly through their perforated bottom walls for return through the ports, 20, of the baffles, 19. It may be understood that several so called "slivers" or assemblies of fibers will be disposed in the respective troughs, 21, as many as three slivers to each trough if desired, and that as soon as these slivers have been entered in the feed rolls, 15, at the discharge end they will be moving slowly through the troughs, 21, for treatment by the heated water therein. The temperature will be maintained between 200° F. and 212° F. by means of the live steam in the pipes, 24, and the convection currents set up in the tank, 14, as already described will serve to insure the treatment of the fiber by substantially the whole mass of water in the tank rather than by any localized portion of it, as might be the case if the water were merely standing in the troughs, 21. This treatment of the fiber by the heated water tends to dissolve away the tannin and chlorofyll and other water soluble substances associated with the fiber at the same time it softens the gum and resinous material rendering it relatively plastic. If the process is continuous the water in the tank or vat, 14, may be changed periodically or continuously by the introduction of fresh water, as through a supply valve, 25, the excess water overflowing the end wall, 26, of the tank, into a short open compartment, 27, having an outlet, 28, which may lead into the sewer or to any suitable receptacle if it is desired to recover the dissolved matter from the water. A drain plug, 29, may also be provided near the bottom of the partition wall, 26, for use in occasionally flushing out the entire tank, 14, at which times any resinous matter which has settled in the tank may be collected and removed.

The fiber will not be injured by treatment with the hot water for a longer period than thirty-five minutes. Therefore the initial portion of the fiber may be allowed to lie in the troughs, 21, this length of time and then may be started through the feed rolls, 15. These rolls are held toward each other under adjustable spring pressure as indicated in Figure 2 and to accommodate the sliver form in which the fiber is being handled, it may be preferable to provide one of said rolls with circumferential grooves, 15a, aligned with the several troughs, 21, and providing space for the thicker portions of the sliver so that substantially equal pressure may be exerted by each of the rolls upon all the fibers of each sliver. This pressure serves to squeeze off from the fiber the major portion of the gum which has been softened and loosened by the hot water treatment in the vat, 14, and this gummy material with the water which is also pressed out by the rolls, 15, is discharged into a special accumulating trough, 28a, and thence through any suitable conduit, 29a, may be car-

ried off for reclamation in accordance with well understood methods. In the process of squeezing the hot-water-saturated sliver between the spring-pressed rolls, the rolls are exposed to the 5 hot water by their contact with the sliver.

Whatever length of "sliver" it is possible to make from the initial quantity of fiber in the receptacle, 13, it will be understood that the sliver may be rendered continuous by splicing onto it 10 from time to time additional units of fiber as delivered from the picker, 8, and before the trailing end of the sliver has entered the trough of the tank, 14. It should also be understood that in the structure as illustrated with multiple 15 troughs, 21, a plurality of these slivers will be started simultaneously and will continue to travel parallel to each other through the apparatus. The fiber continues its movement through the rolls, 15, and enters the second set of troughs, 20 30, in a tank, 31, these troughs and tanks being structurally similar to the troughs, 21, and their tank, 14. The bath in the tank, 31, however, is a weak solution of sodium carbonate, preferably 25 about three percent, and for this reason the exposed metal of this structure should be of copper or heavily nickled to prevent corrosion and to prevent discoloration of the fiber which might occur if ordinary iron piping and tanks were used. The fiber travels through the troughs, 30, 35 at the same rate as it moved through the troughs, 21. As a matter of convenience, if each set of troughs is made about thirty-five feet long the fiber will be moved through them at the rate of one foot per minute. And to avoid cooling and 40 hardening of the gum during the transfer of the fiber from the tank 14 to tank 31, it may be subjected to hot water sprays at 15<sup>a</sup>, and 15<sup>b</sup> adjacent the squeezing rolls, 15, as shown in Figure 2.

40 The function of the alkaline bath of sodium carbonate is to remove any remaining gum from the fiber by dissolving it, thus freeing any associated resin from the fiber and permitting it to fall to the bottom of the vat from which it may 45 be collected at intervals for reclamation in merchantable form. A small quantity of the alkaline solution may be added from time to time to compensate for evaporation and for that which is carried off with the gum and resin removed in 50 the vat, 31. At the end of the tank, 31, the fiber again passes through squeezing rolls shown at 32 which remove most of the alkaline solution from it. These rolls may be mounted directly in the 55 end of the vat, 31, or, as shown, may be separated from it and provided with a collecting trough, 33, for the solution squeezed from the fiber. As the fiber approaches the rolls it may be further clarified by a rinsing spray of clear water indicated at 34.

60 For certain uses such as the manufacture of paper, it is desirable that even the small quantity of alkali remaining in the fiber be neutralized, and for this purpose it may be passed from the rolls, 32, directly into a neutralizing bath of 65 weak acid indicated at 35. Brief dipping in this bath is all that is necessary, therefore the tank, 35, may be of much less length than the preceding tanks employed in the process and from it the fiber may be passed through wringing rolls, 70 36, and then through a rinsing bath of clear water, 37, to final squeezing rolls, 38, which will press most of the moisture from the fiber. Emerging from the rolls, 38, it proceeds across any suitable feed table or support, 39, to a dryer which 75 is indicated diagrammatically in Figure 3 as a

continuous belt conveyor, 40, which may be understood as of any suitable reticulated form, as for example, a series of belts or ribbons with transverse supporting bars secured to them at intervals. Associated with the dryer belt, 40, are 5 suitable heating means such as steam pipes, 41, and a blower, 42, for supplying air through a distributing conduit, 43, with ports, 44, through which the air passes for heating contact with the pipes, 41, and thence through the conveyor belt, 10 40, for drying the fiber. At the discharge end of the belt, 40, the fiber is preferably passed through a series of fluted rolls, 45, which may be similar to the rolls, 3, 4, 5, 6, employed at the beginning of the process except that they need 15 not have corrugations of graduated dimensions, as in the other series, but may be all substantially alike; the function of these rolls, 45, is simply to mildly flex the fiber at the completion of the drying to soften it and loosen from it any 20 film of foreign material which may have adhered through the various washings and rinsings; and may have been dried onto the surface in the final step of the process.

As it emerges from the softening rolls, 45, the 25 fiber may be further treated by combing or carding devices of any suitable design, as may be readily understood by those skilled in the art. It will then be baled for shipment to the user.

For some uses, as for packing or wicking, 30 where the matter of color is not important, the acid dip in the tank, 35, may be omitted and the water in the tank, 31, may be relied upon to sufficiently wash out the alkali from the fiber. Where the matter of color is of vital importance, as in 35 spinning, it may be desirable to subject the fiber to final chemical bleach, but this can be extremely mild by reason of the fact that the material has already been so thoroughly cleansed and washed in the process herein described. As a result, the 40 spinning fiber will be much stronger than that which has been subjected to a relatively severe bleaching, as such process always acts to weaken the cellular structure and therefore tends to weaken the strength of the fiber. Fiber produced 45 in accordance with my process having been degummed almost entirely by mechanical means which at the same time is designed to handle the fiber always gently throughout the process, will be found to present a softness of texture and 50 a luster almost rivaling a silk fiber, and since it has been thoroughly washed and cleared, it will take a fast dye rendering it suitable for spinning and manufacture into cloth for a wide range of 55 purposes for which linen has not heretofore been thought suitable.

In the apparatus shown, as indicated in Figures 2 and 5, I have included vapor hoods, 14<sup>a</sup>, extending slightly above the side walls, 17, of the tanks and communicating with the suction passages, 60 14<sup>b</sup>, so as to draw off steam and other vapors tending to rise from the surface of the liquids in the tanks, thus facilitating handling of the material if necessary by workmen and keeping the premises clear of unpleasant steam and odors. 65 Another feature of construction of the apparatus which is quite important is the provision of oiled pressure pads of absorbent material such as felt or the like shown at 58 in contact with upper and lower rolls of each pair of squeezing rolls for the 70 purpose of cleaning the rolls of any adhering particles or fiber which would otherwise cling to their surfaces by reason of the gum and resin associated with the fiber. These pads serving to coat the rolls with a thin film of oil will prevent ad- 75

hesion of the material and will also act as scrapers to remove fiber which might otherwise be carried around the rolls.

Although I have shown and described herein

- 5 a specific group of mechanisms and apparatus for performing the process and have indicated certain modes of treatment, it is to be understood that the process and apparatus described are illustrative and that my invention is not specifically limited thereto except as indicated by the appended claims; it being evident that various changes and modifications both in the process and the apparatus may be made without departing from the spirit and scope of the invention.

15 I claim:

1. A process for the purpose indicated which includes forming the fibrous material into a sliver after the shive has been removed therefrom and feeding it slowly through a heated water bath 20 to soften the gum and resin and dissolve out the water-soluble material, passing the sliver between rolls for removing the softened gum and resin and protecting the sliver against atmospheric cooling by spraying it with hot water in its passage to and 25 through the rolls.

2. A process for the purpose indicated which includes loosening the shive or woody material from the fiber in its dry state and separating a substantial portion of the said material therefrom, then submerging the fiber for soaking it in liquid maintained at a temperature suitable for softening the gum and resin, and directing a liquid current maintained at said temperature into impact with the sliver while the latter is free 35 from mechanical pressure and without substantial time interval between the submergence of the fiber for soaking it and its exposure to the impact of the liquid current; whereby the gum is maintained in said softened condition throughout the 40 step of separation by liquid current impact.

3. A process for the purpose indicated which includes forming the fibrous material into a sliver after the shive has been removed therefrom, feeding the sliver slowly through a bath of water 45 maintained at a temperature suitable for softening the gum, exposing the sliver to the direct impact of a current of water maintained at said temperature without substantial intermission in the exposure to liquid maintained at said gum-softening temperature and while exposed to said liquid current impact, passing the sliver between squeezing rolls the surfaces of which make contact with the surfaces of the sliver for squeezing, the surfaces of the rolls being thus exposed to said liquid.

- 55 4. A continuous process for the purpose indicated which consists in feeding dry stalks or straw through instrumentalities adapted to apply pressure and limited flexure thereto for loosen-

ing the shive or woody material, and then continuing the movement through a picker arranged for combing out and removing most of said woody material, forming into a sliver the fibrous portion of the straw emerging from the picker and feeding said sliver longitudinally at a relatively slow rate through a liquid bath maintained at temperature suitable for softening the gum, then without intermission in the exposure of the sliver to the liquid maintained at said gum-softening 10 temperature, passing the sliver between squeezing rolls in direct contact of the fiber with the surface of the rolls on opposite sides of the sliver while maintaining the sliver in exposure to the liquid maintained at said gum-softening temperature, splicing additional fibrous material from the picker to the sliver at intervals to extend the length indefinitely, feeding the sliver after passing the rolls into a mild chemical water bath through which it moves longitudinally at the same 20 rate of speed to permit the remaining gum to be dissolved and the associated resin to be freed from the fiber, then feeding the fiber through additional pressure means, rinsing and drying it, and finally subjecting said fiber to mechanical flexure 25 for softening it, and to combing or carding means for removing any adhering particles and straightening the fiber.

5. A process for the purpose indicated which includes forming the fibrous material into a sliver 30 after the shive has been removed therefrom and feeding it slowly through a heated water bath to soften the gum and resin and dissolve out the water soluble material, feeding the sliver out of said bath and then passing it between rolls for 35 dislodging the gum and resin while applying heat to protect the sliver against atmospheric cooling during its passage to and through the rolls.

6. A process for the purpose indicated which includes forming the fibrous material into a sliver 40 after the shive has been removed therefrom and feeding it slowly through a heated water bath to soften the gum and resin and dissolve out the water soluble material, feeding the sliver out of said bath, then subjecting it to mechanical pressure to dislodge the gum and resin and applying heat to the sliver immediately upon its emergence from the heated water bath to prevent cooling and hardening of the gum before its dislodgement.

7. A process for the purpose indicated which includes forming the fibrous material into a sliver 50 after the shive has been removed therefrom, subjecting the fiber to a heated liquid bath to dissolve out the coloring matter and soften the gum and resin, then separately dislodging and collecting the softened gum and resin outside said liquid bath while applying heat to prevent cooling and hardening of the gum and resin.

ROBERT FORSYTH.